

June 26, 1928.

1,674,958

R. S. DEAN ET AL

ALLOY

Filed June 21, 1924

Fig. 1.



Fig. 2.



Inventors  
Reginald S. Dean  
William E. Hudson  
by H. S. Atkinson Atty.

Patented June 26, 1928.

1,674,958

## UNITED STATES PATENT OFFICE.

REGINALD SCOTT DEAN AND WILLIAM EWART HUDSON, OF OAK PARK, ILLINOIS, AS  
SIGNORS TO WESTERN ELECTRIC COMPANY, INCORPORATED, OF NEW YORK, N. Y.,  
A CORPORATION OF NEW YORK.

ALLOY.

Application filed June 21, 1924. Serial No. 721,482.

This invention relates to improved alloys. By improvement in alloys is meant increase in hardness and the like which is secured by the treatment known as age-hardening.

Heretofore, alloys having three or more constituents, such as duralumin, a composition of aluminum, silicon, copper and magnesium have been improved by age-hardening. Such a process, however, has not been successfully applied to binary alloys. Nor has means been provided for obtaining improvement in a particular metallic alloy except the old method of continued trial, commonly called the "cut and try" method.

The object of this invention is to provide improved binary alloys.

The process by means of which the improved binary alloys embodying the invention may be produced, consists in adding to a metal another metal or pseudo metal which will form a solid solution with the first-mentioned metal, the two constituents being of such a nature that the solute is more soluble at one temperature than another, forming a solid solution of the resulting alloy by heating and then quenching and aging the alloy. A marked improvement is obtained by employing the greatest amount of solute which is soluble in the solvent metal at any temperature at which the resulting alloy is a solid, other steps of the process, including heating, quenching and aging, being controlled in a manner which will be explained more in detail hereinafter.

Other features and objects of the invention will appear from a consideration of the following description, and will be particularly pointed out in the appended claims.

In the attached drawing,

Fig. 1 is a graphic curve showing the relationship of solubility of antimony in lead at various temperatures, to the improvement obtainable in lead alloyed with various percentages of antimony; and

Fig. 2 is a similar curve plotted on these characteristics of lead-tin alloys.

This invention is based primarily on the discovery that metallic alloys can be improved by age-hardening when they are of such a nature that one of the constituents is

soluble in the other while in the solid state and when the solubility changes with change in temperature, and that a marked improvement is obtained by employing the amount of solute which is soluble in the carrier metal at the temperature at which maximum solubility occurs.

In carrying out the process the proper proportions of the materials to constitute the alloy, (these proportions being determined as described in the preceding paragraph) are raised to and maintained at a temperature sufficiently high to form a solid solution thereof, the alloy then being quenched to form a supersaturated solution and finally allowed to age until the alloy has assumed a substantially stable state.

A detailed description will now be given of the mechanics of the process and the manner in which it may be performed. It has been found in practicing the process that the following variables are present which have an effect upon the improvement attainable in any particular alloy.

1. Composition of the alloy.
2. Temperature of heating.
3. Time of heating.
4. Size of the mass heated.
5. Shape of the mass heated.
6. Temperature from which quenched.
7. Temperature of quenching bath.
8. Temperature during aging.
9. Time of age treatment.

Each of these variables will now be taken up individually and be discussed in relationship to the other variables.

1. *Composition of the alloy.*—It is often found in considering any particular binary alloy which is of such a nature that one of the materials is soluble in the other, that greater solubility is obtained at one temperature than at other temperatures. For instance, as pointed out in our copending application Serial No. 690,716, filed February 5, 1924, antimony is more soluble in lead at the eutectic fusing temperature than at any other point. Any alloy which shows a greater solubility of its solute constituent at higher temperatures than at lower temperatures and while the alloy is in the solid state, may be age-hardened, and a marked improvement is obtained by employing the

maximum amount of solute constituent which is soluble in the solvent metal while the alloy is in the solid state, or, as stated in another way, by employing the maximum amount of solute which will enter into solid solution with the solvent metal.

A study of the curves shown in the attached drawing will show more clearly the relationship of solubility to hardness.

10 Fig. 1 is a composite graph showing a tensile strength curve superimposed over a solubility curve which is shown as a dotted line. The figures on the right of the graph show the centigrade temperature at which 15 varying percentages of antimony, calibrated on the lower line are soluble in lead. The solid line represents increase in tensile strength by age-hardening. The figures on the left hand margin represent improvement indicated in terms of tensile strength, and the relationship of the improvement to the 20 antimony content may be seen by comparing the dotted solubility curve and the solid tensile strength curve.

25 As is indicated by the position and shape of the two curves the maximum improvement in tensile strength indicated at A is slightly over 7,000 lbs. per square inch and this improvement is obtained by employing 30 about 2.45% antimony with pure lead in the compounding of the alloy. The dotted line indicates that at between 245° C. and 250° C. the maximum solubility of antimony in lead while in the solid state is 2.45%, corresponding precisely with the amount which, 35 other steps of the age-hardening process being properly carried out, causes a marked improvement.

40 In Fig. 2 the dotted line indicates the solubility of tin in lead while in the solid state, and the solid line indicates improvement in terms of micro-Brinell-hardness for varying percentages of tin. The tin content is read from the base line for both curves. 45 The temperatures at which various percentages of tin are soluble are read from the right hand margin, while the Brinell hardness is indicated on the left hand margin. Point B indicates the maximum improvement obtained and is analogous to the point 50 A in Fig. 1. It will be observed that if the tin content is read on the lower line from the point B, the figure 14.5 is obtained and this, as the dotted line indicates, is approximately the limit of solid solubility of tin in lead at any temperature at which the alloy is a solid. These figures show that the percentage of maximum solubility and the percentage of maximum improvement coincide, 55 that the maximum amount of tin soluble in solid lead is about 14.5% and that the greatest improvement by age-hardening is obtained by employing about 14.5% tin and 85.5% lead.

60 The hardness of this material was deter-

mined by means of a micro-Brinell machine using a one-sixteenth inch ball, and a two kilogram weight.

2. *Temperature of heating.*—To obtain maximum improvement the temperature employed during the heating of the alloy must be a temperature at which all of the solute material employed will enter solution. For instance, if 97.55 parts of lead are alloyed with 2.45% antimony, which is about the maximum amount of antimony which will enter solid solution, the alloy must be heated at a temperature slightly below the eutectic fusing temperature. If a percentage of solute is employed which will enter solution at another temperature than that of maximum solubility, another temperature may be employed to obtain the improvement possible with the amount of solute constituent employed. It has been determined, however, that if the maximum percentage of solute is not employed, no harm will come from heating the material at the temperature at which the maximum solubility occurs. In carrying out an age-hardening method, therefore, it is advisable and desirable to employ as near as possible in the heating step the temperature at which maximum solubility occurs. For most metallic alloys this will mean heating at a temperature slightly below the eutectic fusing temperature.

3. *Time of heating.*—To obtain desirable results the heating is preferably carried on for a sufficient length of time to obtain a perfect homogeneous solid solution. Although the percentage of material that will enter into solution may be said to be a certain amount, where differential solubility is observed at various temperatures, it invariably takes some time to obtain a homogeneous solid solution with that amount of solute at the temperature employed. For instance, as shown in our copending application referred to above, the percentage of antimony which is soluble in lead at 240° C. is about 2.45%. Supposing the temperature is in accordance with the requirements stated in the previous paragraph, in order to obtain a perfect solution with this percentage of antimony it is necessary to heat the alloy sometimes as long as 72 hours before homogeneity is obtained.

105 This is an important step in the treatment of age-hardened alloys because if a perfect homogeneous solid solution is not obtained the improvement of the metal may be very adversely affected.

110 4. *Size and shape of the mass heated.*—If one of the constituents be appreciably lighter in weight than the balance of the alloy, it has a tendency to rise to the top when the molten alloy is cast into a mold. 115 As an example, antimony is considerably lighter than lead and it has been observed 120

that it will rise to the top of a mold, particularly if a large casting is poured or if the shape of the casting is such that certain portions will project up considerably above other portions. This rising of a light constituent is termed segregation and is observable particularly in large sized castings. If there has been great segregation due to the size and shape of the casting, the time of 10 heating must be lengthened. The segregation is not a matter which is of prime importance in the process which is the subject-matter of this invention. The important step, the composition being determined, 15 is obtaining solid solution. Segregation simply lengthens the time required for solid solution to form at the temperature employed.

6. *Temperature from which quenched.*— 20 In order to obtain the best results the material should be quenched while in a state of solid solution. This means that quenching must take place at about the temperature which is necessary to obtain solid solution, 25 that is, the temperature of the heating step. However, if the material enters into solution quite slowly, it will usually be found to stay in solution and separate out quite slowly. When this is the case quenching may take 30 place at a slightly lower or higher temperature than the temperature at which the first heating is carried on.

7. *Temperature of the quenching bath.*— 35 The purpose of quenching is to quickly change the temperature of the material to bring it to its normal temperature without permitting a change in the lattice or structure of the material itself, that is to say, the material is retained in substantially the same 40 condition as it was in at the higher temperature. Quenching, therefore, may be accomplished in any manner which will have this result. For many alloys, for example lead-antimony, quenching can be effected by 45 means of water at room temperature.

8. *Temperature during aging.*—Aging may take place at any temperature which will allow sufficient molecular movement in the material to accomplish the age-hardening. 50 In general, aging can be accomplished more quickly at a higher temperature than at a lower temperature. It is also generally the case that aging should not take place at a high enough temperature to permit annealing of the alloy which it is sought to age. The critical temperature is usually termed the temperature of recrystallization. It has been found that in order to secure high tensile strength and hardness it is advantageous to age the alloys at temperatures at 55 which the solute constituent precipitates from the supersaturated solution in a finely divided form, or in other words, at a temperature low enough to insure little agglomeration of the precipitated particles. Since

the particles are precipitated from a substantially homogeneous solid solution at such a low temperature that little agglomeration occurs, they are substantially uniformly dispersed throughout the solvent material and are much smaller in size than the agglomerated particles produced by other methods of treating binary alloys.

9. *Time of age treatment.*—The time required for aging a particular alloy will vary with the temperature. Some age-hardened alloys will continue to show an increased hardness or improvement over a long period of time. For instance, lead antimony alloys will show a very great hardening after 72 hours aging at room temperature. It is observable, however, that even after a matter of months, they will continue to harden gradually. This after-hardening effect, however, is not great, but it shows the amount of time that must sometimes be allowed before the maximum aging will have taken place and likewise will be definitely concluded. If, however, the preliminary steps, that is, the composition requirements, time and temperature of heating, temperature from which quenched and temperature to which quenched, are such as to cause a maximum hardness, the aging will have the effect of causing maximum hardness in time, even if it is materially retarded on account of the employment of too low a temperature.

The subject-matter of the present invention can be applied not only to binary alloys which show the characteristics described, but also to alloys which may be referred to as pseudo-binary alloys. An example of this type of alloy is lead, copper and antimony, particularly when certain percentages are employed. As an example, a small percentage of copper added to lead-antimony has the effect of causing increased solubility of the antimony in lead. The amount of antimony soluble in lead at the eutectic fusing temperature is about 2.45%. When .1% of copper, however, is added, this is increased to 3.25%. The same process which is applied to the ordinary binary alloys, having the properties referred to, can also be applied to such an alloy as lead, copper and antimony. The process constituting the present invention may also be applied to certain binary alloys in which one of the constituents is not directly soluble in the other. As an example, an alloy wherein two metals form compounds in definite proportion and then the compound becomes soluble in the majority member of the alloy may be subject to treatment by the same method.

Where a solid solution is formed in metals, it is very difficult to determine whether the solute metal goes into solution directly with the carrier material, or whether a chemical compound is formed and the compound then goes into solution in the carrier material.

Where a solid solution is formed and reference made to such "solid solution" in either the description of the invention or the appended claims, it is intended to include in the term "solid solution" either type of solution. It is immaterial from the standpoint of the present invention what the type of solute material is, improvement by age-hardening independent of the underlying theory being the subject-matter of the invention. It will be noted from a study of the hardness and tensile strength curves in the attached figures that there is some latitude over which desirable results are obtained. Each one of the curves is partially flat on top, and the composition indicated by reading from the center of the flat portion represents the greatest improvement. It is not desired, however, to limit this invention to a method for obtaining the hardness resulting by employing the percentage of alloying matter shown on a representative curve as the point equivalent to the point A in Fig. 1. We have determined that a variation of about 20% in volume of the solute material will not cause any great departure from the desired improvement. In the appended claims, therefore, "substantially" has been employed to describe a departure of about 20% from the maximum amount

of solute material soluble in the carrier material.

Although reference has been made throughout to specific applications of the process, it is to be understood that such reference is not meant to be a restriction, but that the invention is to be limited only by the scope of the appended claims.

What is claimed is:

1. A lead-antimony alloy in which lead is the major constituent, characterized by the presence of finely divided particles of antimony substantially uniformly dispersed throughout the lead. 40

2. A lead-antimony alloy containing the greatest amount of antimony which will enter solid solution in lead at any temperature, and characterized by the presence of finely divided particles of antimony substantially uniformly dispersed throughout 50 the lead. 45

3. A lead-antimony alloy containing from 1 to 2.5% antimony, and characterized by the presence of finely divided particles of antimony substantially uniformly dispersed 55 throughout the lead. 50

In witness whereof, we hereunto subscribe our names this 7th day of June, A. D., 1924.

REGINALD SCOTT DEAN.

WILLIAM EWART HUDSON.